

# UNITED STATES PATENT OFFICE.

JUDSON A. DE CEW, OF MOUNT VERNON, NEW YORK, ASSIGNOR TO PROCESS ENGINEERS INCORPORATED, OF NEW YORK, N. Y.

## ENGINE-SIZING FOR PAPER.

1,401,525.

Specification of Letters Patent. Patented Dec. 27, 1921.

No Drawing.

Application filed August 24, 1921. Serial No. 495,097.

*To all whom it may concern:*

Be it known that I, JUDSON A. DE CEW, a citizen of Canada, residing at Mount Vernon, New York, have invented certain new and useful Improvements in Engine-Sizing for Paper, of which the following is a specification.

This invention relates to the sizing of paper pulp in the beating engine and it consists essentially in coagulating resin with alum in the presence of a coagulated colloid.

The ordinary process of sizing paper pulp in the beating engine consists in adding a rosin soap to the paper pulp and then coagulating this by means of sulfate of aluminum, or alum.

I have discovered that the properties of this rosin and alumina precipitate are altered and improved if a coagulation of other colloidal materials takes place in the presence of one of these ingredients and before the other is added.

The method I prefer to follow in obtaining this result is to bring the rosin soap to a dilute solution in water in the presence of mucilaginous material, and an agent which has a coagulating effect upon the mucilaginous product.

*Example.*—A rosin soap containing about 2% of glue is dissolved in water to form a 1% solution of rosin, and sufficient formaldehyde is added to make the glue insoluble in the water. This mixture is then added to the paper stock in the beating engine where the rosin soap is coagulated by the sulfate of aluminum.

Another way to carry out this process is to add the rosin size and mucilaginous material to the beating engine where they will be dissolved and mixed together and then to coagulate first the mucilaginous or gluey matters by the addition of formaldehyde solution and then to rosin size with alum.

The result of this process is a mixture of

sizing materials which will resist the injury 45 to sizing usually experienced in machine drying, and which will give a better finish to the paper. By mucilaginous materials, I mean glue, gelatin, casein, starch products, natural gums in the paper stock, and the 50 like.

Whereas I have mentioned formaldehyde as the coagulating agent I may use tanning substances, or other coagulating agents so long as they coagulate the mucilaginous or 55 colloidal substances but do not precipitate the size.

What I claim is:

1. A paper size consisting of a dilute solution of rosin soap in water containing a 60 colloidal material coagulated therein.

2. A paper size consisting of an approximately 1% solution of rosin soap, glue and formaldehyde in water.

3. A process of making a paper size 65 which consists in dissolving a rosin soap and a colloidal material into water and then adding a product which will coagulate the colloidal material and not the soap.

4. A process for making a paper size 70 which consists in making a dilute solution of rosin soap containing glue and adding sufficient formaldehyde to render the glue insoluble.

5. A paper size which consists of a rosin 75 soap containing a non-resinous colloidal material, in a highly diluted aqueous solution, the colloidal material having been coagulated while in the dilute condition.

6. A process of making a paper size 80 which consists in dissolving a rosin soap and a colloidal material into water to form a dilute solution and then adding a reagent which will coagulate only the non-resinous material.

In testimony whereof I have affixed my signature to this specification.

JUDSON A. DE CEW.